

N. TESTRUP AND T. RIGBY,  
BY-PRODUCT RECOVERY FROM GAS PRODUCERS AND THE LIKE,  
APPLICATION FILED MAR. 7, 1916.

1,316,339.

Patented Sept. 16, 1919.



INVENTORS:

Nile Testrup,  
Thomas Rigby.

By Byers, Townsend & Brinkertbine, ATTORNEYS.

# UNITED STATES PATENT OFFICE.

NILS TESTRUP, OF WESTMINSTER, LONDON, ENGLAND, AND THOMAS RIGBY, OF DUMFRIES, SCOTLAND.

## BY-PRODUCT RECOVERY FROM GAS-PRODUCERS AND THE LIKE.

1,316,339.

Specification of Letters Patent. Patented Sept. 16, 1919.

Application filed March 7, 1916. Serial No. 82,656.

*To all whom it may concern:*

Be it known that we, NILS TESTRUP, a subject of the King of Great Britain and Ireland, and residing at 3 Dean Farrar street, 5 Westminster, London, S. W., England, and THOMAS RIGBY, a subject of the King of Great Britain and Ireland, and residing at 61 Loretburn street, Dumfries, Scotland, have invented certain new and useful Improvements in and Relating to By-Product Recovery from Gas-Producers and the like, of which the following is a specification.

This invention relates to the recovery of by-products in the gasification of peat, coal 15 and other fuels in gas producers and the like having a distillation and a combustion zone.

In such processes, the tar is usually separated from the liquor and sold, to be thereafter worked up by tar distillers, who distil 20 off various oils and obtain pitch as a residue. In the majority of cases such pitch contains about half its weight of volatile matter, while the harder varieties contain as much as 30 to 40 per cent. thereof. Hitherto it has 25 not been practicable to obtain pitch of a good quality containing none of such volatile matter, as further coking of the material in the stills requires such a high temperature as to produce decomposition of the pitch, and render 30 the stills liable to damage.

We have found, however, that the pitch, whether of the medium or hard quality, can be readily distilled without the over cracking of the gases and deposit of fixed carbon 35 accompanying distillation in a retort by introducing it into a producer along with the ordinary raw fuel supply thereto, and that the greater portion of the volatile matter is then given off as an oil-bearing tar, and 40 is recovered with the tar emanating from the raw fuel itself. In this way, the amount of tar recovered from the producer and the quantity of oil obtained from the tar stills is proportionately increased, while the non-volatile portion of the pitch consisting 45 mainly of carbon is converted first to carbon dioxide and then reconverted into carbon monoxide in the lower part of the producer until nothing remains but ash, which is discharged in the usual manner. By thus utilizing the pitch, the revenue from by-products is substantially increased.

It is to be understood that the invention does not relate to the distillation of pitch 55 in closed or like retorts in which no subse-

quent combustion of the residual carbon and other substances is effected, nor does it apply to the spraying of liquid pitch directly into the combustion zones of gas producers or furnaces.

The invention consists, therefore, in distilling the residual pitch from the tar stills in the distillation zones of a solid fuel body such as that of a producer.

The invention also consists in the process 65 for the utilization of peat in which the peat tar is distilled, and the residual pitch passed directly into the gas producers, from which the power needs of the process are supplied.

The invention further consists in the improved methods for distilling pitch as hereinafter described.

In the arrangement shown by way of example in the accompanying drawing, the tar is distilled in the still A and the pitch is run 75 off into pitch cooling ponds B. After cooling, the pitch is broken in the pitch breaker C and conveyed by means of a suitable elevating or conveying device D to bunkers E, whence it is fed in measured quantities by 80 means of a measuring device F into a hopper H over the gas producer J. The fuel is fed by means of the elevating device K, hopper E<sup>1</sup> and measuring device F<sup>1</sup> into the producer hopper H, the speeds of the two 85 measuring machines being preferably set so that the mixture in the hopper H contains fuel and pitch in definite proportions. The mixed pitch and fuel is then fed into the producer J and the volatile constituents of 90 the pitch are distilled by the heat of the producer gas in the distillation zone of the producer J passing over with the producer gas into the tar washer L whence these products are washed out from the gases which 95 then pass away by means of the main M for use.

The carbon constituents of the pitch pass downward into the combustion zone of the producer where they are gasified together 100 with the carbon of the fuel.

When operating in accordance with the invention care must be taken in the arrangement that the pitch is completely distilled before the residue reaches the zone of combustion and in order to achieve the foregoing result the pitch is mixed as intimately as possible with the fuel, either in the manner described or in the liquid form by spraying. In the former case, the pitch is prefer- 105

60

70

75

80

85

90

95

100

105

110

- ably broken into pieces about the size of an egg, or of such size as to be uniform with the particles of fuel by which the gas producer is fed.
- 5 The depth of the gas producer is preferably so arranged that the distillation of the pitch is complete before the residue reaches the combustion zone, which results in a high proportion of the volatile matter 70 distilled from the pitch being carried forward in the producer gas as condensable products. The final result is that the tar, which is condensed from the gas in the tar extracting apparatus gives a higher yield 10 of oil than is produced under ordinary conditions. Consequently when such tar is distilled in the distillation plant, a much higher proportion of oil is given off than is the case with tar normally produced from the fuel.
- 15 It has been found that the tar deposited in the various parts of the tar recovery apparatus of the producer plant, is of a more oily nature and has the additional advantage that in an ammonia recovery plant of 80 this type, the oily nature of the tar washes and purifies the sulfate liquor.
- 20 The tar so recovered from the sulfate liquor tanks is in a thinner condition than usual, and is therefore more easily separated 85 from the sulfate liquor, and with a much less loss of sulfate than is the case under ordinary conditions.

It will be seen that many other advantages besides increased yield of oil are obtained 35 by this process, and it is found that the quantity of pitch which can be fed to the producer may be varied within wide limits without detriment, although a constant rate of feed should preferably be maintained 40 when once fixed upon, so that the fuel proper may be intimately mixed in regular proportions with the pitch.

When working with peat fuel the tar normally produced gives off about 50 per cent. 45 oil in distillation, 45 per cent. being pitch and 5 per cent. being wasted by decomposition, &c., in the distillation. The addition of this pitch to the producer in this cycle of operations results in the fact that nearly one-half as much oil again is produced. This means that from 100 parts of tar (calculated dry) 70 parts of oil as end product are obtained. It is also found that the nitrogen in the pitch after distilling in the producer is 55 higher than in the original fuel from which the pitch came. In one case in which the fuel contained 11 $\frac{1}{2}$  per cent. nitrogen, the pitch coke after distillation by this system showed 2 per cent. nitrogen with the result 60 that in an ammonia recovery gas producer, the yield of ammonia is greater from this than from a corresponding weight of normal fuel.

When working with coal, in one case, the 65 tar normally produced gave on distillation

20 per cent. of the original bulk of tar (calculated dry) as oil, 75 per cent. being pitch and the remainder being lost in decomposition in the stills. When this pitch is fed to the gas producer in the correct ratio it is 70 found that the yield of oil per ton of tar (calculated dry) becomes approximately from 50 per cent. to 55 per cent. of the original weight of tar, the remaining 45 per cent. being gasified as pitch-coke in the gas 75 producer in the usual manner.

In the case of blast furnaces using coal, the same principles may be applied as above, and the oil yield correspondingly increased with the result that there is no pitch containing 80 large percentages of ash to be disposed of, and the utilization of the fuel value of the pitch-coke means a saving in the amount of fuel used in the blast furnace, while at the same time the more valuable commodity, oil, 85 is produced in correspondingly greater quantities.

In feeding pitch into the blast furnace it may be fed in intimate admixture with the other charging materials or the pitch 90 may in the first place be amalgamated with any of the ingredients of the charge for the furnace, care being exercised that it is introduced in such a manner that the whole of the volatile matter has been distilled from 95 the pitch in the distillation zone before the residue can reach the zone of combustion. This applies in all cases, whether to blast furnace or gas producer apparatus, as it has been found that if the pitch is allowed 100 to reach the combustion zone it is burnt and consumed to gases instead of forming oil, as might be expected.

In the case of gas producers in which the fuel is more or less caking and in which 105 there is a tendency for cracks to form in the fire, it is preferred that the pitch be fed into the producer in such a manner that it tends to remain largely in the center part of the producer as by this means there is 110 not the same tendency for the pitch when it becomes liquid to run through the cracks to the combustion zone, the pitch not being in active contact with the producer gases being made, and being more or less distilled 115 in the more stagnant parts of the fuel bed.

Having now described our invention, what we claim as new and desire to secure by Letters Patent, is:—

1. A method of utilizing pitch consisting 120 in gasifying the volatile and non-volatile constituents thereof in a gas producing chamber through which it moves to successively hotter zones in admixture with other matter such as fuel and in the reverse direction to air admitted to said chamber.

2. A method of utilizing pitch consisting 125 in gasifying the volatile and non-volatile constituents thereof in successive temperature zones of a gas producing chamber to 130

which it is fed in admixture with other matter such as fuel, said chamber being heated by partial combustion of part of the mixture.

5 3. A method of utilizing pitch consisting in gasifying the volatile and non-volatile constituents thereof in successive temperature zones of a gas producing chamber heated by partial combustion therein of the 10 non-volatile portions of said pitch and other fuel with which it is mixed.

4. A method of utilizing pitch consisting in feeding said pitch homogeneously mixed with other matter such as fuel to the upper 15 portion of a furnace chamber, distilling said pitch by the heat of gases generated by combustion taking place under regulated air supply in the lower portion of said chamber and finally completing the combustion 20 of said pitch in said lower portion of the chamber.

5. A method of utilizing pitch consisting in incorporating it in a mixture containing fuel such as peat, coal or other combustible

matter adapted to retain its solid character 25 while burning, and passing the mixture through a chamber in which progressively increasing temperature zones are maintained for the purpose of gasifying the volatile and non-volatile constituents of the pitch.

30 6. A method of utilizing pitch consisting in incorporating it in a mixture containing fuel such as peat, coal or other combustible matter adapted to retain its solid character 35 while burning, and passing the mixture through a chamber in which progressively increasing temperature zones are maintained by partial combustion of part of the mixture.

In testimony whereof we have signed 40 our names to this specification.

NILS TESTRUP.  
THOMAS RIGBY.

Witnesses:

A. BROWN,  
A. P. OBHOH,  
J. E. DEXTER,  
J. KELLY.

Copies of this patent may be obtained for five cents each, by addressing the "Commissioner of Patents.  
Washington, D. C."